# EUROPEAN PATENT APPLICATION

(11) **EP 2 055 494 A1**
(43) Date of publication of application: **06.05.2009**
(21) Application number: 07119762.8
(22) Date of filing: 31.10.2007
(51) Int. Cl.: B41M 3/14, B41M 7/00, B42D 15/00

(54) **Copy protected paper**

(71) Applicant: Nederlandse Organisatie voor Toegepast- Natuurwetenschappelijk Onderzoek TNO, 2628 VK Delft (NL)
(72) Inventor: Hovens, Irene Antoinette Petra, 5913 CD Venlo (NL); Batenburg, Lawrence Fabian, 5652 EJ Eindhoven (NL); Timmermans, Johannes Wilhelmus, 6714 GG Ede (NL); Rentrop, Cornelis Hermanus Arnoldus, 5616 AE Eindhoven (NL); Jetten, Jan Matthijs, 3701 JL Zeist (NL); Turkenburg, Daniël Hendrik, 5643 DM Eindhoven (NL)
(74) Representative: Hatzmann, Martin

(57) **Abstract**

The invention is directed to copy protected paper, to a method for producing said paper, the use of a specific coating for copy protection of paper, and a method for protecting a printable paper substrate from being copied.

The copy protected substrate of the invention comprises a printable substrate having, on a printed side, a transparent coating comprising an organic polymer, wherein the refractive index of said transparent coating differs from the refractive index of said substrate with at least 0.1.

## Description

The invention is directed to copy protected paper, to a method for producing said paper, and a method for protecting a printable paper substrate from being copied.

Paper is used as a medium for recording all kinds of printed information. Normally such information can be copied, for instance by means of a photocopier. However, in particular when the information contained on the paper is valuable (such as in the case of banknotes, cheques, licences, certificates, paper with copyright information, or other security paper) it is not desirable that the original can easily be copied.

In the prior art several attempts have been made to protect a paper original from being copied. Some of these attempts are directed at adjusting photocopiers, others are directed at using special inks or toners, still others are directed at the use of specific printing technologies. It would, however, be desirable to have a paper that is protected against making copies. Ideally, the copy of such a paper would be unreadable or unrecognisable. However, it would already be advantageous to be able to immediately distinguish the copy from the original.

JP-A-2004 188 950 describes a paper having a black camouflage pattern printed thereon. A layer of fluorescent ink is provided on top of the black camouflage pattern. Information printed on this paper can be read by irradiating the paper with black light and the fluorescent layer emits coloured light. A copy of the original turns out black because of the black camouflage pattern. Major disadvantages of this paper are that the original paper has a black colour and that the information on the original can only be read by irradiating the paper with black light.

JP-A-4 201 562 describes a paper on which is provided a resin layer containing transparent fine particles having reflective ability and reflective pigment. Incident light transmits through the transparent fine particles and is reflected by the reflective pigment, which is emitted from the transparent fine particles. Due to the reflective pigment, the resin layer is visible. Furthermore, in order to have the desired effect, a combination of transparent fine particles with the reflective pigment is required.

Object of the invention is to at least partially overcome the disadvantages of the prior art.

Another object of the invention is to protect a paper from being copied using a coating that is not visible.

A further object of the invention is to provide a paper that is protected from copying in that the copy can be immediately distinguished from the original.

Another object of the invention is to provide an accessible and cheap method for protecting printable paper from being copied.

The inventors found that one or more of these objects can be met by providing a substrate with specific refractive index properties.

Accordingly, in a first aspect the invention is directed to a copy protected substrate comprising a printable substrate having, on a printed side, a transparent coating comprising an organic polymer, wherein the refractive index of said transparent coating differs from the refractive index of said substrate with at least 0.1.

The term "copy protected substrate" as used herein refers to a substrate that can contain printed information and of which the copied information is at least significantly different than the original information. Thus, when the original information contained on the copy protected substrate is copied, the information on the copy is at least significantly different than the original information. The copied information can for instance be in the form of a photocopy, but also a scan of the original, for instance by a digital scanner, is considered a copy in the context of this invention.

The copy protected substrate of the invention thus comprises a printable substrate which is printed on at least one side of the substrate. The printed substrate is overlaid with the transparent coating. If desirable, the coating can be printed on.

The difference in refractive index between the transparent coating and the substrate causes the substrate to be copy protected. Information printed on the substrate under the transparent coating is visible under low angles, typically angles of less than 90°, preferably less than 70°, more preferably 70°-50°. However, under substantially right angles, typically angles of 30-90°, preferably angles of 70-90°, more preferably angles of 90°, the information becomes invisible because of total reflection.

In the most extreme form the transparent coating under substantially right angles functions as a mirror and totally reflects the light of a copying device. As almost all copying devices shine light onto the original under right angles or substantially right angles, the substrate is protected from being copied by almost all copying devices.

The difference between the refractive index of the transparent coating and the refractive index of the substrate is at least 0.1. The refractive index can reliably be measured by a refractometer. The wavelength can be varied and is usually measured or expressed in index at 550 nm. In a more preferred embodiment the difference between the refractive index of the transparent coating and the refractive index of the substrate is at least 0.2, preferably at least 0.5, more preferably 0.5-1.0. The larger the difference in refractive index, the wider the angle under which incident light is totally reflected. At very big differences in refractive index, such as differences of more than 1.0, a large extent of light is reflected so that the information on the original becomes hard to distinguish with bare eye. For instance, if the information is in the form of a text, the original may be hard or impossible to read.

In principle the refractive index of the transparent coating can be either lower or higher than the refractive index of the substrate. In practice, it has been found convenient to prepare a transparent coating with a refractive index that is higher than the refractive index of the substrate.

The substrate can be chosen from a wide range of materials. Examples of substrates that can be used in accordance with the invention include different types of paper and fabrics, such as such as bank paper, inkjet paper, photographic paper, wool fabric, silk fabric, cotton fabric, flax fabric, polyester fabric, aramid fabric, acrylic fabric, nylon fabric, and spandex fabric.

In accordance with the invention it is also possible that the substrate is a coated substrate (such as a coated paper). The substrate may be coated with an inorganic coating such as china clay and/or TiO₂. In this case, the refractive index of the transparent coating should differ from the refractive index of the coated substrate with at least 0.2. The transparent coating comprises an organic polymer. In a preferred embodiment the organic polymer is selected from the group consisting of starch, cellulose, polyvinylalcohol and derivatives thereof. Particularly, preferred organic polymers are for instance copolymers of polyvinyl alcohol and polyvinyl acetate optionally with itaconic acid, carboxymethylcellulose, and amylase free potato starch (for instance the amylopectin potato starch Eliane^{™}, commercially obtainable from AVEBE).

The transparent coating of the substrate according to the invention can comprise inorganic particles. If particles are present, these particles should have an average particle size, which is smaller than the wavelength of light in the visible in order to prevent scattering of light, which would make the coating non-transparent. Thus, the particles can have an average particle size of 0.5-200 nm, preferably 0.6-100 nm, more preferably 0.7-50 nm, as determined by transmission electron microscopy.

Inorganic particles can for instance be selected from the group consisting of TiO₂ (refractive index of the particles about 2.2), SnO₂, Si (refractive index of the particles about 4.0), Ag (refractive index of the particles about 1.35), Au (refractive index of the particles about 0.47), C(diamond) (refractive index of the particles about 2.4), ZnO (refractive index of the particles about 2.0), ZrO₂ (refractive index of the particles about 2.2), CeO₂ (refractive index of the particles about 2.3), and Hf₂O₃ (refractive index of the particles about 1.9).

In a preferred embodiment, the transparent coating comprises inorganic particles having a refractive index difference of at least 0.5 compared to the polymer/coating, preferably a difference of at least 1.0, more preferably at least 1.5 as determined with a refractometer. It was found that inorganic particles with a refractive index that strongly differs from the refractive index of the substrate significantly contribute to the copy protection of the substrate.

The inorganic particles can be dispersed in the organic polymer. Preferably, the particles are dispersed homogeneously and the formation of aggregates is prevented. Aggregate formation could lead to an aggregate particle size which is larger than the wavelength of light, thereby causing light scattering and in turn leading to a non-transparent coating. In order to increase the compatibility of the particles with the organic polymer it is possible to modify the surface of the inorganic particles. Typically, the surface of the inorganic particles is modified with organic compounds comprising ammonium, phosphonium, carboxylic, siloxane, and/or hydroxylic groups.

Another possibility to make the inorganic particles more compatible with the organic polymer is to add one or more surfactants to the transparent coating. Suitable surfactants include block-copolymers. Suitable blocks for use in the block-copolymers for instance include polyethylene oxide, maleic acid anhydride, carbonic acid, alcohol, and polyethylene glycol, polypropylene, polyethylene, polystyrene, polymethylmethacrylate, polyamide, and polyethylene oxide. The block-copolymers may be provided with a functional terminus, such as a carbonic acid group, a hydroxyl group, or an epoxy group. It is also possible to combine the addition of surfactants with a surface modification of the inorganic particles.

The amount of the particles in the coating can be chosen in a wide range. It is preferred that the coating comprises 1-50 wt.%, preferably 20-40 wt.%, more preferably 30-40 wt.% of the inorganic particles. The ratio between the inorganic particles and the organic polymer in the transparent coating is preferably at least 5:95, more preferably at least 50:50. When the ratio between inorganic particles and organic polymer in the transparent coating is more than 50:50, this can cause problems in the preparation of the coating. Accordingly, the ratio between the inorganic particles and the polymer in the transparent coating is preferably in the range of 2:98-40:60, more preferably 10:90-20:80. A high amount of inorganic particles compared to the amount of organic polymer may cause problems in viscosity of the coating solution. In addition, such a high relative amount of inorganic particles can lead to less transparent coatings. If the amount of inorganic particles is very low it becomes more difficult to realise a sufficiently high difference in refractive index with the substrate.

In a special embodiment of the invention, the inorganic particles are quantum dots (semiconductor nanoparticles), which are optionally fluorescent.

The transparent coating may further comprise one or more dyes. The dyes can be inorganic, organic, or a mixture of inorganic and organic dyes can be used. Suitable organic dyes are for instance acridine dyes, anthraquinone dyes, diarylmethane dyes, triarylmethane dyes, azo dyes, phtalocyanine dyes, diazonium dyes, quinone dyes, azin dyes, indamine dyes, indophenol dyes, oxazin dyes, oxazone dyes, thiazin dyes, thiazole dyes, xanthene dyes, fluorene dyes, rhodamine dyes, and fluorone dyes. The inventors found that the provision of a dye in the transparent layer can cause an additional show-through effect during copying of the original, i.e. when information is provided on both sides of the original, the single-sided copy contains the information of both sides of the original.

Without wishing to be bound by theory, it is believed that the show-through effect of the invention relates to a spectral overlap of the absorption of the dye in the transparent layer with the emission spectrum of the lamp of the photocopying machine or scanner. It is believed that the show-through effect increases when this spectral overlap is increases.

Therefore it in a preferred embodiment, the transparent layer comprises a dye which has an absorption spectrum that overlaps with the emission spectrum of the lamp of the photocopier.

If one or more dyes are included, it is preferred that the dyes are strongly absorbing. The dye can have for example a molar extinction coefficient at its absorption maximum of at least 10 000 Lmol⁻¹cm⁻¹, preferably at least 20 000 Lmol⁻¹em⁻¹, more preferably at least 50 000 Lmol⁻¹cm⁻¹. In practice there are only few dyes with a molar extinction coefficient of more than 200 000 Lmol⁻¹cm⁻¹.

In a special embodiment, the transparent coating comprises one or more emitting dyes, preferably fluorescent dyes. Suitable fluorescent dyes include fluoresceins, rhodamines, coumarins, and the like. Also phosphorescent dyes can be used. Irradiation by a lamp of a photocopying machine can bring the emitting dye in an excited state after which the dye can emit light, either by fluorescence or by phosphorescence. This emitted light can interfere with the photocopying process. Fluorescent dyes are preferred over phosphorescent dyes, because fluorescence is a faster relaxation process than phosphorescence.

When the transparent coating comprises emitting dyes, it is preferred that the transparent layer is provided with means to concentrate the emitted light. Such means can for instance be grooves or pits in the transparent layer. Such grooves or pits in the transparent layer should have a dimension larger than the wavelength of the emitted light. It was found that such grooves or pits can efficiently concentrate the emitted light, thereby increasing the interference with the photocopying process. The grooves or pits, which are hardly visible in the original because of their small size (typically smaller than 100 µm, preferably smaller than 50 µm), appear in the copy as bright areas as a result of the interfering emitted light.

For very thin layers the observed total reflection effect becomes small. In such cases a copy of the information printed on the substrate may not be not unrecognisable, but still distinguishable from the original. Preferably, the transparent coating on the substrate preferably has a layer thickness of at most 1 000 nm, preferably at most 500 nm, more preferably at most 200 nm. The layer thickness can be reliably measured by a profilometer. It is in general difficult to fabricate coatings with a layer thickness of more than 5 µm. In a preferred embodiment, the transparent coating has a layer thickness of 100-500 nm.

In a further aspect the invention is directed to a method of preparing a copy protected substrate as described above, comprising
- providing a printable substrate;
- printing information on a side of said substrate;
- providing a coating composition comprising an organic polymer, which coating composition, when dried, has a refractive index that differs at least 0.1 from the refractive index of said printable substrate;
- applying said coating composition to a printed side of said substrate; and
- drying said coating composition.

The coating solution can simply be prepared by mixing the components together in a suitable mixing process. Optionally, solvents can be added. Suitable solvent for instance include water, alcohols (such as ethanol, pronanol, isopropanol, butanol, and the like), ketones (such as aceton, methylethylketone, and the like). Subsequently, the coating composition is applied to the printed substrate. This can be performed by any coating method known in the art, such as air knife coating, immersion (dip) coating, gap coating, curtain coating, rotary screen coating, reverse roll coating, gravure coating, metering rod (meyer bar) coating, slot die (extrusion) coating, or hot melt coating. At least the printed side should be coated in accordance with the method of the invention, but it is also possible to coat more than one side of the substrate.

As mentioned above it is also possible that the substrate is a coated substrate (such as a coated paper). This coated substrate can be printed on, and subsequently the printed substrate can be overlaid with the transparent coating. In this case, the refractive index of the transparent coating should differ from the refractive index of the coated substrate with at least 0.1 after drying and more preferably 0.2 or higher.

In a further aspect the invention is directed to a method of protecting a printed substrate from being copied comprising applying on the substrate, on the printed side, a transparent coating as defined above.

In yet a further aspect the invention is directed to the use of a transparent coating as defined in any one of claims 1-10 as a copy protection for information printed on a substrate.

The copy protected paper of the invention can be used for copy sensitive information, such as the information on paper money, banknotes, cheques, licences, certificates, vouchers, tickets, papers with copyright information, or any other security paper.

### Examples

### Example 1- TEOS (coating solution 1 (25 % w/w))

10.86 g TEOS (tetraethoxysilane) and 22.84 g IPA (isopropylalcohol) was mixed at 0 °C (ice bath) for 15 minutes while adding dropwise 4.4 g 1 M HNO₃ and 1.7 g of demineralised water. Next this solution was refluxed at 80 °C for 2 hours. This solution is mentioned as the stock solution 1 (25 % w/w).

### Example 2- TEOS (coating solution 2 (2.5 % w/w))

Coating solution 1 was diluted with IPA to obtain a concentration of 2.5 % (w/w).

### Example 3 - TEOS (coating solution 3 (0.25 % w/w))

Coating solution 1 was diluted with IPA to obtain a concentration of 0.25 % (wlw).

### Example 4- TIPT (coating solution 4 (25% w/w))

28.42 g TIPT (tetra-isopropoxytitane) was mixed with 100 ml IPA and 10.01 g Acac (2,4-pentadione, acetylacetonate) at 23 °C for 5 minutes in a closed vessel. This solution is mentioned as the stock solution 2 (25 % w/w).

### Example 5- TIPT (coating solution 5 (2.5 % w/w))

Coating solution 4 was diluted with IPA to obtain a concentration of 2.5 % (w/w).

### Dipping procedure

The papers were dipped in the coating solutions attached to a glass plate to prevent wrinkling. The papers were totally submerged for 25 seconds before the dipping process (upward motion) was started.

### Example 6 - TEOS (25 % w/w)

Regular copying paper (79 g/m²) was coated with the coating solution 1 from example 1. The coating was dipped in the stock solution 1 with an upward velocity of 8 mm/s leaving behind 16.7 g/m² of coating. Figure 1 shows the results copied on a Xerox standard copier (black and white). Figure 1A is a digital photo of the original coated paper, Figure 1B is a result of a copied coated paper at high sensitivity.

### Example 7 - TEOS (25 % w/w)

Regular copying paper (79 g/m²) was coated with the coating solution 1 from example 1. The coating was dipped in the stock solution 1 with an upward velocity of 1 mm/s leaving behind 15.4 g/m² of coating. Figure 2 shows the results copied on a Xerox standard copier (black and white). Figure 2A is a digital photo of the original coated paper, Figure 2B is a result of a copied coated paper at high sensitivity.

### Example 8- TEOS (2.5 % w/w)

Regular copying paper (79 g/m²) was coated with the coating solution 2 from example 2. The coating was dipped in coating solution 2 with an upward velocity of 8 mm/s leaving behind 4.1 g/m² of coating. Figure 3 shows the results copied on a Xerox standard copier (black and white). Figure 3A is a digital photo of the original coated paper, Figure 3B is a result of a copied coated paper at high sensitivity.

### Example 9 - TIPT / TEOS (2.5 % w/w; 25 % w/w TEOS)

Regular copying paper (79 g/m²) was coated with the coating solution 5 from example 5. The coating was dipped in coating solution 5 with an upward velocity of 8 mm/s and after drying the coated paper was dipped in coating solution 1 with 8 mm/s. Figure 4 shows the results copied on a Xerox standard copier (black and white). Figure 4A is a digital photo of the original coated paper, Figure 4B is a result of a copied coated paper at high sensitivity.

### Example 10 - TEOS 25 % w/w

Regular photo paper (233.5 g/m²) was dipped in coating solution 1 from example 1 with an upward velocity of 8 mm/s leaving behind 6.1 g/m² of coating. Figure 5 shows the results copied on a Xerox standard copier (black and white). Figure 5A is a digital photo of the original coated paper, Figure 5B is a result of a copied coated paper at high sensitivity.

### Example 11- TEOS 25 % w/w

Regular photo paper (233.5 g/m²) was dipped in coating solution 1 from example 1 with an upward velocity of 1 mm/s leaving behind 3.9 g/m² of coating. Figure 6 shows the results copied on a Xerox standard copier (black and white). Figure 6A is a digital photo of the original coated paper, Figure 6B is a result of a copied coated paper at high sensitivity.

## Claims

1. Copy protected substrate comprising a printable substrate having, on a printed side, a transparent coating comprising an organic polymer, wherein the refractive index of said transparent coating differs from the refractive index of said substrate with at least 0.1.

2. Copy protected substrate according to claim 1, wherein the transparent coating further comprises inorganic particles having an average particle size of 0.5-200 nm, preferably 0.6-100 nm, more preferably 0.7-50 nm.

3. Copy protected substrate according to any one of the preceding claims, wherein the organic polymer is selected from the group consisting of starch, cellulose, polyvinylalcohol, and derivatives thereof.

4. Copy protected substrate according to any one of the preceding claims, wherein the refractive index of the transparent layer is at least 0.2 higher, preferably at least 0.5 higher, more preferably 0.5-1.5 higher than the refractive index of the substrate.

5. Copy protected substrate according to any one of claims 2-4, wherein the inorganic particles are selected from the group consisting of TiO₂, SnO₂, Si, Ag, Au, C(diamond), ZnO, ZrO₂, CeO₂, and Hf₂O₃.

6. Copy protected substrate according to any one of claims 2-5, wherein the coating comprises 1-50 wt.%, preferably 20-40 wt.%, more preferably 30-40 wt.% of inorganic particles.

7. Copy protected substrate according to any one of the previous claims, wherein the transparent coating has a layer thickness of at most 1 000 nm, preferably at most 500 nm, and more preferably at most 200 nm.

8. Copy protected substrate according to any one of claims 2-7, wherein the inorganic particles have a refractive index of at least 0.4, preferably at least 1.0, more preferably 1.0-4.0, and most preferably 2.0-4.0 as determined by a refractometer.

9. Copy protected substrate according to any one of claims 2-8, wherein the surface of the inorganic particles is modified with one or more organic compounds.

10. Copy protected substrate according to claim 9, wherein said one or more organic compounds comprise ammonium, phosphonium, carboxylic, siloxane, and/or hydroxylic groups.

11. Copy protected substrate according to any one of the previous claims, wherein the substrate is chosen from the group consisting of paper (such as bank paper, inkjet paper, photographic paper), natural fabric (such as wool fabric, silk fabric, cotton fabric, and flax fabric), and synthetic fabric (such as polyester fabric, aramid fabric, acrylic fabric, nylon fabric, and spandex fabric).

12. Copy protected substrate according to any one of the previous claims, wherein said transparent coating comprises one or more dyes.

13. Copy protected substrate according to claim 12, wherein said dye is an organic dye selected from the group consisting of acridine dyes, anthraquinone dyes, diarylmethane dyes, triarylmethane dyes, azo dyes, phtalocyanine dyes, diazonium dyes, quinone dyes, azin dyes, indamine dyes, indophenol dyes, oxazin dyes, oxazone dyes, thiazin dyes, thiazole dyes, xanthene dyes, fluorene dyes, rhodamine dyes, and fluorone dyes.

14. Copy protected substrate according to claim 12 or 13, wherein said dye is an emitting dye.

15. Method of preparing a copy protected substrate according to any one of claims 1-14, comprising
- providing a printable substrate;
- printing information on a side of said substrate;
- providing a coating composition comprising an organic polymer, which coating composition, when dried, has a refractive index that differs at least 0.1 from the refractive index of said printable substrate;
- applying said coating composition to a printed side of said substrate; and
- drying said coating composition.

16. Method of protecting a printed substrate from being copied comprising applying on the substrate, at least on the printed side, a transparent coating as defined in one of claims.

17. Use of a transparent coating as defined in any one of claims 1-14 as a copy protection for information printed on a substrate.
